

## UNITED STATES PATENT OFFICE

2,017,167

## PHOTOGRAPHIC DEVELOPER

Harold D. Russell, Rochester, N. Y., assignor to  
 Eastman Kodak Company, Rochester, N. Y., a  
 corporation of New York

No Drawing. Application August 1, 1934,  
 Serial No. 737,958

4 Claims. (Cl. 95—88)

This invention relates to photographic developers, and more particularly to developers in which the usual alkalies are replaced by a compound new for the purpose.

5 Alkaline developers have been known and used for many years. These developers usually contain developing agents, a so-called preservative, such as sodium sulfite, and an alkali, such as sodium or potassium carbonate, or sodium or potassium hydroxide. In recent years various sensitive materials and photographic processes have appeared with which the use of these relatively strong alkalies is objectionable for one reason or another. One object of this invention  
 10 is to provide developers containing a milder alkali. Another object is to provide developers which will give satisfactory results without the objectionable features of those containing the alkalies previously used, such as the formation  
 15 of gas blisters when a film developed in a developer containing carbonate is immersed in an acid fixing bath.

20 I have discovered that by using a sodium salt of triethanolamine as the alkaline component, developers may be prepared which fulfill all these objects.

25 The sodium salts of triethanolamine may be prepared by dissolving powdered sodium hydroxide in triethanolamine, with heating. The amount of sodium hydroxide used is one, two or three equivalent weights, depending upon whether the mono-, di- or tri-sodium salt of triethanolamine is desired. The three salts, or mixtures thereof, may be used interchangeably in developer formulae.

30 Suitable developer formulae embodying my invention are given here, by way of example.

## EXAMPLE 1

|                                |    |       |
|--------------------------------|----|-------|
| 40 Hydroquinone                | 10 | grams |
| Sodium sulfite                 | 10 | do.   |
| Potassium bromide              | 5  | do.   |
| Sodium salt of triethanolamine | 50 | do.   |
| 45 Water to make               | 1  | liter |

## EXAMPLE 2

## TWO-BATH FORMULA

## Bath No. 1

|                  |     |       |
|------------------|-----|-------|
| 50 Elon          | 5   | grams |
| Hydroquinone     | 10  | do.   |
| Sodium sulfite   | 100 | do.   |
| Sodium bisulfite | 5   | do.   |
| 55 Water to make | 1   | liter |

## Bath No. 2

|                                |    |       |
|--------------------------------|----|-------|
| Sodium sulfite                 | 10 | grams |
| Sodium salt of triethanolamine | 50 | do.   |
| Water to make                  | 1  | liter |

5 The film or plate is first immersed in Bath No. 1 for 2 to 3 minutes and then in Bath No. 2 until development is complete.

## EXAMPLE 3

|                                |      |       |
|--------------------------------|------|-------|
| Elon                           | 5    | grams |
| Hydroquinone                   | 10   | do.   |
| Sodium sulfite                 | 75   | do.   |
| Sodium salt of triethanolamine | 50   | do.   |
| Potassium bromide              | 5    | do.   |
| Potassium iodide               | 0.01 | do.   |
| Water to make                  | 1    | liter |

## EXAMPLE 4

|                                |      |       |
|--------------------------------|------|-------|
| Elon                           | 5    | grams |
| Hydroquinone                   | 10   | do.   |
| Sodium sulfite                 | 75   | do.   |
| Sodium salt of triethanolamine | 20   | do.   |
| Potassium bromide              | 5    | do.   |
| Potassium iodide               | 0.01 | do.   |
| Water to make                  | 1    | liter |

20 The above examples show the sodium salt of triethanolamine as the sole alkaline component of the developer. I have found, however, that mixtures of a sodium salt of triethanolamine 30 with other alkalies are advantageous for some purposes. For example, I may use a mixture of caustic soda, borax, and a sodium salt of triethanolamine. Or I may use a mixture of sodium metaborate and a sodium salt of triethanolamine. Following is an example of a developer 35 in which such a mixture of alkalies is used.

## EXAMPLE 5

|                                |    |       |
|--------------------------------|----|-------|
| Elon                           | 2  | grams |
| Hydroquinone                   | 5  | do.   |
| Sodium sulfite                 | 50 | do.   |
| Sodium metaborate              | 30 | do.   |
| Sodium salt of triethanolamine | 10 | do.   |
| Potassium bromide              | 2  | do.   |
| Water to make                  | 1  | liter |

40 It will be understood that I am not to be limited by the above examples except as indicated in the appended claims.

45 While I have spoken of the sodium salts of triethanolamine, it will be apparent that I may also use the potassium or other alkali metal salts of triethanolamine.

50 What I claim as my invention and desire to 55

be secured by Letters Patent of the United States  
is:

1. A photographic developer comprising a de-  
veloping agent and, as an essential alkaline-re-  
acting component of the developer, an alkali  
metal salt of triethanolamine.
2. A photographic developer comprising a de-  
veloping agent and, as an essential alkaline-re-  
acting component of the developer, a sodium salt  
10 of triethanolamine.

3. A photographic developer comprising a de-  
veloping agent and an alkali, at least 25%, ap-  
proximately, of the alkali consisting of an alkali  
metal salt of triethanolamine.

4. A photographic developer comprising a de-  
veloping agent and an alkali, at least 25%, ap-  
proximately, of the alkali consisting of a sodium  
salt of triethanolamine. 5

**HAROLD D. RUSSELL. 10**